

# UNITED STATES PATENT OFFICE.

GEORGE D. VAN ARSDALE, OF NEW YORK, N. Y.

## ART OF CONCENTRATION OF ORES BY FLOTATION.

1,236,504.

Specification of Letters Patent. Patented Aug. 14, 1917.

No Drawing.

Application filed February 7, 1916. Serial No. 76,757.

To all whom it may concern:

Be it known that I, GEORGE D. VAN ARSDALE, a citizen of the United States, residing at New York, in the county of New York and State of New York, have invented certain new and useful Improvements in Art of Concentration of Ores by Flotation, of which the following is a specification.

My present invention is an improvement 10 in the art of concentration of ores by flotation and relates particularly to the preparation of the ores to insure their proper concentration by flotation.

It has been known that oxidized 15 pounds of metals, for example, copper, are not readily concentrated by the ordinary flotation methods, but that such oxidized copper compounds may be converted into sulfids in various ways, and thereby rendered capable of being concentrated by flotation. One method of converting such oxidized compounds into sulfids is by introducing hydrogen sulfid into a pulp containing the ore to be concentrated in a finely divided 20 state. The result of this treatment is a more or less complete conversion of the oxids into sulfids, the extent of this conversion being in some cases merely a film, and in others a more complete conversion, depending on the 25 fineness of the mineral, the amount of hydrogen sulfid present, and other factors. For practical purposes a complete conversion is more desirable than a film, for the reason that for the flotation of many ores it has been found necessary to add the oils during 30 the milling operation. It is obvious that a film of sulfid even of quite an appreciable thickness, will not be resistant to milling but will be abraded from the core of oxid, the 35 practical result being an incomplete extraction. In order to obviate this, it is necessary to add an excess of hydrogen sulfid, but it has been found that it is very difficult to add just the exact amount required for the 40 conversion of the copper, and that an excess of free hydrogen sulfid above such an amount is very detrimental to flotation.

It is necessary therefore to provide means for rendering such excess harmless in practical work, and such a means is described in these specifications and constitutes an improvement in the art.

I have heretofore spoken of copper ores, and will describe this improvement as applied to such ores, but it can be readily understood that the same methods will apply

to ore other than copper, and I do not wish to confine the scope of this improvement therefore to copper ores only.

In experimenting with certain copper 60 bearing materials, for example, slime tailings, in which a considerable part of the copper is in the oxidized condition, I have found that the amount of hydrogen sulfid necessary for complete conversion of such 65 oxids into sulfids, is not excessive, for example, in one class of material the amount needed is from 120% to 140% of the theoretical amount calculated from the amount of oxid copper present. I have also found 70 that there is a more or less preferential action of such added hydrogen sulfid on the copper minerals present. That is to say, the oxidized copper compounds are first converted into sulfid, while there are still left 75 remaining other constituents of the pulp capable of combining with free hydrogen sulfid.

I have found therefore that in order to convert all of the copper present into sulfid 80 compounds it is necessary to add at least the excess determined by assay on the material being treated to be necessary. Since practically this excess cannot be controlled exactly but can be controlled within certain limits, 85 I have found that the amount of hydrogen sulfid added must be kept within the amount that can be absorbed by the other constituents of the pulp capable of reacting with hydrogen sulfid, and that when kept below this 90 limit the excess will be readily neutralized and rendered harmless.

I have also found that the element of time enters into the operation, that is to say, it is necessary to allow sufficient time first for the 95 conversion of the oxids, and second to allow sufficient time for the absorption and neutralization of the excess hydrogen sulfid by the other constituents of the ore being treated.

This invention therefore consists in the discovery that a practical method of concentration as above outlined depends on the addition to the pulp of an amount of hydrogen sulfid sufficient to convert all of the 105 oxid copper present to sulfid, together with an additional amount of the reagent not in excess of the amount that can be absorbed and neutralized by the pulp, and of the fact that such excess, which has been found detrimental hitherto may be rendered harmless, 111 first by controlling the amount as above, and

secondly by allowing a certain amount of time for its absorption and neutralization to take place.

With a pulp treated as outlined above it is possible to get good concentration results by flotation, but without this method or other methods of rendering the excess hydrogen sulfid harmless, good results are not obtained.

10 Other methods have been described for accomplishing this end, for example, by the introduction of sulfur dioxid into the pulp after treatment by hydrogen sulfid. It is obvious however that the method described 15 is radically different from this, and while accomplishing the same results, is much simpler and cheaper.

In carrying out this invention, the following apparatus and procedure may be used 20 and followed, although of course modifications of both may be made.

The necessary steps of the operation are as follows, after suitable preliminary grinding, etc., of the material to be treated.

- 25 1. Generation of hydrogen sulfid.
2. Absorption of hydrogen sulfid by the pulp.
3. Time of standing.
4. Flotation.

30 Practically the hydrogen sulfid may be generated in any suitable way dependent on local conditions. One suitable method will be by the action of acid on low-grade copper iron matte, carrying say about 10% of copper. The undissolved residue from the action of the acid on such matte will contain all of the copper, gold and silver present, and may accordingly be recovered and treated by smelting, thus reducing the cost of 40 the necessary hydrogen sulfid.

The hydrogen sulfid may be brought into contact with the pulp in a closed vessel provided with means of agitating the pulp and with means for continuous supply and discharge of the pulp, and of continuous supply of the gas, which may preferably be under slight pressure. By suitably adjusting the supply and discharge of pulp and of gas to this vessel the amount of hydrogen sulfid 50 needed may be kept within proper limits as described above, and as determined by assay in each individual case.

After treatment in this apparatus, the pulp may be conducted to another apparatus 55 to allow time for the complete absorption of the excess of gas. This apparatus may be simply a closed tank, provided with means for agitation. Ordinarily from two to four hours' time will be found sufficient to absorb 60 and neutralize all excess hydrogen sulfid.

After this step the pulp may be treated exactly as in ordinary flotation, that is to

say, by addition of oil or other necessary reagent, and the operation of flotation carried out in any of the ordinary apparatus for the 65 purpose.

In addition to the treatment of ores in which a part or all of the minerals present are as oxids, the process will be found applicable to other ores whose minerals have a 70 film of oxid only covering them. Ordinarily such ores are treated either by sufficient attrition to mechanically remove such films or by the addition of acid or both. When acid is added the amount needed is an important factor in the cost of flotation, and it is believed that treatment of such ores by the method described above will be cheaper and give a better recovery than by the methods ordinarily in use, particularly 80 where considerable amounts of acid are used.

Having thus described my invention, what is claimed as new is:

1. The process of separation by flotation of the mineral and the gangue constituents 85 of an ore which consists in supplying hydrogen sulfid to the ore bearing pulp to an amount in excess of the amount required for combination with the non-sulfid mineral present, in letting the pulp so treated stand 90 until the excess hydrogen sulfid has been absorbed, and in then separating the mineral and the gangue by flotation.

2. The process of separation by flotation of the mineral and the gangue constituents 95 of an ore which consists in adding hydrogen sulfid to the ore bearing pulp in such quantity that it may all be utilized in combining with the mineral and other ingredients of the pulp, the quantity being in excess of the 100 quantity for the mineral present, and in then separating the mineral and the gangue by flotation.

3. The process of separation by flotation of the mineral and the gangue constituents 105 of an ore which consists in bringing hydrogen sulfid into contact with the pulp while the latter is agitated, in then permitting the pulp to stand, the quantity of hydrogen sulfid employed being in excess of the amount 110 required for the proportion of mineral in the pulp, and in then separating the mineral and the gangue by flotation.

4. The process of separation by flotation of the mineral and the gangue constituents 115 of an ore which consists in supplying hydrogen sulfid to the ore bearing pulp, in letting the ore so treated stand until all free hydrogen sulfid has been absorbed, and in then separating the mineral and the gangue by 120 flotation.

In testimony whereof I affix my signature.